

Dec. 12, 1939.

B. GASPAR

2,183,394

PHOTOGRAPHIC MATERIAL AND PROCESS FOR THE PRODUCTION OF MULTICOLOR PICTURES

Filed July 27, 1937

FIG. 1.



FIG. 4.



FIG. 2.



FIG. 5.



FIG. 3.



FIG. 6.



xxxxx = sensitization.

= absorption.

= screened by overlying layer.

INVENTOR.

*Bela Gaspar,*

BY *F. Gerald Foye*

ATTORNEYS.

## UNITED STATES PATENT OFFICE

2,183,394

PHOTOGRAPHIC MATERIAL AND PROCESS  
FOR THE PRODUCTION OF MULTICOLOR  
PICTURES

Béla Gaspar, Brussels-Forest, Belgium

Application July 27, 1937, Serial No. 156,031  
In Germany March 24, 1932

15 Claims.

(Cl. 95—2)

This invention relates to a photographic recording material for the production of multicolor images and more particularly to a multi-layer material in which one or more colorless light sensitive layers are combined with light sensitive layers which contain dyestuffs. If desired, the colorless layers may contain dyestuff forming substances which are converted into dyestuffs later on in the process of producing multicolor pictures. The present application is a continuation-in-part of my prior applications Ser. No. 662,396 filed Mar. 23, 1933 and Ser. No. 1,437 filed Jan. 11, 1935.

The use of colored light sensitive layers in a multi-layer photographic material has many advantages over the use of a colorless multi-layer material, the layers of which have to be selectively dyed after exposure in order to obtain a multicolor image. The principal advantage is the ease with which each of the light sensitive emulsions may be uniformly predyed before it is coated on the support, as compared to the difficulty of selectively dyeing the various colorless emulsion layers on the support after they have been exposed.

It will be understood that if all of the layers of the exposure material are colored, part of the visible light is absorbed at the surface of the front layer and therefore cannot produce a silver image in the layer. It is, for this reason, out of the question to record all of the visible light spectrum from one side of a multi-layer exposure material in which all of the layers are predyed and the absorption characteristics of said dyestuffs overlap to produce more or less complete absorption throughout the visible spectrum. In practice, it is possible to confine the absorption resulting from the coloration of the front layer to a narrow range of the spectrum so as not to substantially impair the correct reproduction of a natural color. On the other hand, it is desirable to avoid this absorption during exposure and to allow all of the visible light to be utilized in the formation of the image.

In my Patent No. 1,985,344, December 25, 1934, I have disclosed an exposure material for the production of multicolor images in which all of the layers are uniformly dyed with dyestuffs used later on in the process for the formation of the color image, the layers being inseparably superimposed to form a multi-layer photographic material. In my prior patent, the dyestuffs used in the various layers are so selected that a previous gap remains, thus allowing light to penetrate the sensitized layer and to produce a silver image therein. By this arrangement all of the layers of the material may be exposed from one side.

According to the present invention, the necessity of dyeing the layers with dyes having gaps

in their absorption characteristics is avoided by employing an exposure material, in which part of the light sensitive layers are colorless so that all of the exposure light can be recorded from one side.

As pointed out above, the colorless front layer or layers may contain dyestuff forming substances which can subsequently be converted into dyestuffs or these layers may be subsequently colored by any well known coloring process. In such a material it is possible to expose all of the layers of the multi-layer exposure material, so as to obtain color separation images of the original subject in silver. Since part of these layers are already predyed and the colorless layer or layers may contain dyestuff forming substances or may be subsequently dyed, multicolor master images may thereafter be obtained by selectively removing or forming the dyestuff under the influence of the color separation images composed of silver. In converting the silver images into color images, I may proceed, for example, as set forth in my prior Patents 1,956,017, April 24, 1934; 2,020,775, November 12, 1935; and 2,004,625, June 11, 1935.

It is therefore an object of my invention to provide a multi-layer photographic material having both colorless and colored sensitized layers, which material is adapted to record all of the visible exposure light from one side.

In the practice of my invention I do not need to use dyes for the colored layers which are complementary to the sensitivities of said layers, nor do I need to use dyes which are the same as the sensitivities of these layers. This departure from previous lines of endeavor leads to the production of a multicolor image which does not reproduce the original subject in its natural colors. Such an image may be used as a master image from which multicolor copies can be made, reproducing the subject in its natural colors. A copying material suitable for use in this connection is described and claimed in my copending application Serial No. 642,960, filed November 16, 1932. The color sensitization of the single layers in the copying material is complementary to the colors of the corresponding layers in the master image. Thus, by using the proper colors in the corresponding layers of the copying material a final image may be obtained therein which is a reproduction in natural colors. It is also possible to use a copying material such as disclosed in my prior Patent No. 1,985,344, December 25, 1934, wherein three differently colored and differently sensitized layers are poured one on the other.

The exposure material of the present invention is preferably in the form of a multi-pack material. It is therefore possible to separate at least one of the layers from the others so that it may later be used independently for copying.

purposes. For example, it is possible to expose one of the inseparably superimposed and pre-dyed layers of a copying material from the back while the other layers of the copying material are exposed from the front. By this arrangement, I have permitted a much greater liberty with respect to the sensitization of the inseparably superimposed layers of the copying material. Also I have provided a flexible arrangement of colors and sensitivities both in the exposure material and in the copying material. For example, the single layer of the exposure material which is adapted to be separated from the others may be dyed blue-green, sensitized to record the blue part picture, and may be used in the copying process to expose a red sensitized yellow dyed layer. On the other hand the same single layer of the exposure material may be dyed magenta, sensitized to record the same blue part picture, and may be used to expose a green-sensitive yellow dyed layer of the copying material. The choice of these two alternatives depends upon the color of the layer above the yellow dyed layer in the copying material. For example, if the upper layer contains a green absorbing dyestuff transmitting red, the single layer of the exposure material will be dyed blue-green, as set forth first above.

It is therefore a further object of my invention to provide an improved exposure material having colored layers, in which the color of the pre-dyed layers is independent of the color of the separation image which it is desired to record in said layer.

In accordance with the present invention, I have also found that since I am not limited in the selection of the dyestuffs in the colored layers, I may so select them as to do away with the necessity for filter dyestuffs in certain layers during exposure, which dyestuffs have later to be washed out. To do this I impart to these dyestuffs a dual function, namely, the function of acting as a filter for the layer in which they are incorporated, as well as for the layer situated thereunder, and also the function of remaining in the layer to produce a dyestuff image corresponding to the silver image. Thus the dyestuff present in an overlying layer screens the underlying layer against light rays to which it may be sensitive, but which it is not desired to record therein, and the underlying layer is therefore effectively insensitive to these rays.

Accordingly, it is a further object of my invention to provide a multi-layer photographic material having colored layers in which the dyestuffs in the colored layers act both as a filter and as an image-forming material.

In the accompanying drawing, Figure 1 illustrates diagrammatically the relative absorption characteristics and sensitivities of the layers in the preferred embodiment of my invention. Figure 2 represents a similar diagrammatical illustration of a different arrangement of absorption characteristics and relative sensitivities. Figure 3 represents a similar diagrammatical illustration of still another embodiment of my invention. Figure 4 represents a diagrammatical illustration of the relative absorption characteristics and sensitivities of the layers in a typical copying material for use in conjunction with my exposure material. Figure 5 and Figure 6 refer to diagrammatical illustrations of the relative absorption characteristics and sensitivities of the layers in a modification of my invention, wherein the light sensitive layers are in a more close contact.

Referring to Figure 1, which is exemplary of a section through a multi-layer photographic material in which three different layers I, II and III are combined with two supports A and B, the transparent support A carries on the front thereof a colorless blue-sensitive, i. e., not specially sensitized, layer I. On the rear of the support A is a yellow low-dyed green sensitive layer II. On the front of support B is a red-dyed red-sensitive layer III. The supports A and B may consist, for example, of Celluloid or acetyl cellulose.

On the cross-section illustrated in Figure 1, I have projected a spectrum which commences at the left of the figure with the infra-red rays and extends over the entire visible spectrum. The vertical lines which cut all of the layers show, as indicated by the legends, the wave lengths. For example, the legend 600 m $\mu$  indicates approximately the line of separation between the red and green spectral zones, and the legend 500 indicates approximately the separating line between the green and blue spectral zones. The obliquely shaded areas indicate the absorption curves of the dye used to color the layer. The vertically shaded zones indicate that the exposure light which penetrates the material from the surface of the layer I, is screened by the absorption of an overlying layer. The x's in the figure indicate the range of the spectrum with respect to which the particular layer is sensitive. Thus, for example, it is seen in Figure 1, the colorless front layer I is sensitive for the blue spectral zone. Layer II is sensitive for the green spectral zone and colored by a yellow dye whose absorption characteristic falls in the blue spectral zone. This dye may be, for example, chrysophenine G, 304 Schultz dyestuff tables, and the layer may be sensitized with respect to green, for example, with benz-thio-pseudocyanin ethiodide. This yellow dye acts on the one hand as a filter by absorbing the blue rays transmitted by the colorless front layer I and also serves later on in the process for the formation of a color image. Layer III is sensitized in the red spectral zone for example, for pinacyanol, and colored red with a dye whose absorption characteristic falls in both the green and blue spectral zones. This dye may be, for example, Diamine Fast Pink P (no index number) or anthosine BN (referred to by Pier-David in "Kunstliche Organische Farbstoffe", page 663, published by Julius Springer, Berlin, 1926). Thus, layer III is light absorbing in the blue spectral zone, and, in addition to this, it is screened from the exposure light in the blue spectral zone by reason of the blue absorption characteristic of the yellow dye in the overlying layer II. Furthermore, due to the green absorption, in layer III, it is effectively insensitive in the green spectral zone even though it might have some natural sensitivity therein.

In Figure 2, the arrangement of the layers Ia, IIa and IIIa, with respect to the supports A and B, is the same as in Figure 1. Layer Ia is colorless and has the same sensitivity as layer I in Figure 1. Layer IIa likewise has the same sensitivity and color absorption characteristic as layer II in Figure 1. The dyestuff and sensitizer used in this layer may be the same as that used in layer II of Figure 1. In layer IIIa, a yellow dye is used having the same absorption characteristic as the yellow dye used in layer IIa. This may be a yellow dyestuff such as chrysophenine G, the same as the dyestuff used in layer IIa. Thus layer IIIa has an absorption characteristic in the

blue spectral range as well as being shaded in the blue spectral range by the yellow dyestuff in the overlying layer IIa. Layer IIIa is sensitized for the red spectral zone, the same as layer III in Figure 1, and is effectively insensitive to blue due to the blue absorption of the overlying yellow layer II, as well as yellow dye in the layer itself.

Figure 3 shows a relative arrangement of dyestuffs and sensitivities practically the same as in Figure 1. The only difference in this respect is that in IIIb, I have illustrated a dyestuff having an absorption characteristic in the green spectral zone, for example, a magenta dyestuff. This layer IIIb differs from layer III in that the absorption characteristic of the dyestuff does not extend through the green and blue spectral zones, and this layer, instead of being light-absorbing in the blue spectral zone, is merely screened by the blue absorption of the yellow dyestuff in the overlying layer IIb. A suitable dyestuff for layer IIIb is Diamine Fast Pink G or Sirius Ruby. The main difference between Figure 3 and Figure 1 is that the colorless layer Ib is carried on the back of the support A; the yellow-dyed layer IIb is carried on the front of the back support, and the purple red-dyed layer IIIb is carried on the rear of the back support B. Thus, the front film comprising the transparent support A and layer Ib, is an ordinary film with a non-sensitized, i. e., merely blue sensitive, layer and the back film comprising transparent support B with colored layers IIb and IIIb is the only part of the material having predyed layers.

In all of the Figures 1, 2 and 3, the front colorless layer may have incorporated therein, a colorless dyestuff-forming substance which will result in a dyestuff upon subsequent treatment. I may use, for example, a leuco-ester salt of hexabromindigo, such as disclosed in my prior Patent No. 1,956,017, April 24, 1934, or any other desired dyestuff-forming substance.

It is also possible to color the front colorless layer by toning or any other well known process. For example, it may be subsequently colored with a blue dyestuff, for example, Diamine Pure Blue FF, 424 (Schultz dyestuff tables).

It is particularly important that the amounts of the dyestuffs, or the dyestuff-forming substances incorporated in the layers, be exactly determined beforehand in order that one may always obtain in the photographic material an image which is colored to exactly the same degree.

In Figure 4, I have illustrated a cross-section of a typical copying material. This material is a multi-layer material having a support with one layer IV on one side of the support and two layers V and VI on the other side of the support. As indicated in the figure, the layer IV has incorporated therein a blue-green dyestuff, for example Diamine Pure Blue FF. The layer V has incorporated therein a yellow dyestuff, for example, chrysophenine G, and the layer VI has incorporated therein a magenta dyestuff, for example, Sirius Ruby. Layer IV is sensitized in the green spectral region with erythrosine, layer V in the red spectral region with pinacyanol, and layer VI in the blue spectral region.

In copying from a master image produced in the material of Figure 1, onto the copying material illustrated in Figure 4, the front film in Figure 1 is first separated from the back film and the image in layer III is transformed into a red dyestuff image in accordance with the dye

destroying process described in my prior Patent 2,020,775, November 12, 1935. It is then possible to print the red dyestuff image thus produced in layer III, which is carried by support B, into layer IV of the material shown in Figure 4. This is done by printing from the blue-green side of Figure 4, and using a green printing light. Since layer IV is green-sensitive, and since the red image in layer III acts in a shading fashion, one may reproduce in layer IV a silver image corresponding to the red image in layer III. This silver image may later be converted to a blue-green dyestuff image in accordance with the dye destruction processes referred to above. The image originally produced in layer III of Figure 1 was a red color-selection picture and we now have a corresponding part-picture in layer IV of Figure 4 in a complementary color, i. e., blue-green.

After dyeing layer I of Figure 1 by a blue-green dyestuff, such as Diamine Pure Blue FF and after having produced by dye-destruction in layer I of Figure 1 a blue colored image corresponding to the blue color-selection picture therein, and a yellow picture in layer II of Figure 1, the front film with its yellow image in layer II and its blue image in layer I is printed into layers VI and V from the magenta colored side of the material illustrated in Figure 4. Utilizing a white printing light, the yellow image in layer II will influence the blue portion of the printing light which acts on the blue-sensitive layer VI, thus producing a corresponding silver image in this layer. Similarly, the blue image in layer I will influence the red portion of the printing light which acts on the red-sensitive layer V, thus producing a corresponding silver image in layer V. The portion of the printing light falling in the green spectral zone will have no effect since it is absorbed at the surface of layer VI by the magenta dye incorporated therein. By utilizing the color destruction processes, above referred to, a magenta colored image may be produced in layer VI corresponding to the yellow image in layer II. In like manner, a yellow image will be produced in layer V corresponding to the blue image in layer I. Since layer II is green-sensitive, it contains the green color-selection picture which is represented therein by a yellow color and which is reproduced in layer VI in a magenta color. The image recorded in layer VI is therefore seen to be colored complementary to the color-selection picture recorded in layer II. Similarly, the yellow colored part image in layer V is complementary to the blue color-selection recorded in layer I.

The master image produced in the material of Figure 2 may be copied into the printing material, illustrated in Figure 4, in the same way that a master image, according to Figure 1, is copied, except that this time the layer IV of Figure 4 must be made blue-sensitive instead of green-sensitive, in order that the yellow image in layer IIIa will act in a shading fashion when printed into Figure 4 from the top. In such a case, the fact that both layers IV and VI of Figure 4 are blue-sensitive, will cause no difficulty since layers IV and VI are printed from opposite sides of the material and the intervening layer V contains a yellow dye which has an absorption characteristic in the blue spectral range and therefore acts as a blocking layer between layers IV and VI.

In printing a master image produced in the material of Figure 3, the process is carried out in the same way except that layers Ib and IIb

are not printed at the same time, as was the case in connection with layers I and II. The reason for this is that in the modification of Figure 3, layers I<sub>b</sub> and II<sub>b</sub> are carried by different supports and therefore, when the multi-pack is separated, each goes with its respective support. The magenta image in layer II<sub>b</sub> is printed into layer IV of Figure 4 with green light, the yellow image in layer II<sub>b</sub> causing no interference since its transmission characteristic includes green. The yellow image in layer II<sub>b</sub> is printed into layer VI of Figure 4 with blue light, the magenta image in layer II<sub>b</sub> causing no difficulty since its transmission characteristic includes blue.

15. Thus it is apparent that while the multicolor picture reproduced in the exposure material of Figures 1, 2 and 3 is unnatural in the sense that it does not reproduce the colors of the original, nevertheless, the multicolor copy produced in the copying material is a natural and true reproduction, due to the fact that the variations in color of the image in the exposure are compensated for in the copying process. For example, the yellow image produced in layer II by destroying the dyestuff locally in proportion to the silver image, represents the green color sensation of the subject, but the yellow image in layer II is copied into layer VI of the copying material, where it produces a magenta image, thus correctly reproducing the green color-sensation of the original for the subtractive process of producing color pictures. From this explanation the dual function of the yellow dyestuff in layer II is readily understood, since, as pointed out heretofore, it serves as a filter to absorb the blue rays transmitted by layer I and, as above explained, it serves the purpose of an image forming material in layer II.

In carrying out my invention with the embodiments illustrated in Figures 1, 2 and 3, in which the respective photographic layers are separated by a support, it has been found that the images lack sharpness to a certain extent. This difficulty may be remedied by pouring two of the light-sensitive layers one on the other, both being supported on one support. By bringing such a film in face-to-face relation with another film having one light-sensitive layer, we have a bi-pack material in which two layers are in immediate contact with a third single layer. It is possible to unite two bi-pack films having two layers on the one side so that the layers are situated in immediate contact upon exposure. The technical advantage of such an arrangement resides in the fact that the light sensitive layers are situated practically in one optical plane. An additional advantage consists in the fact that a considerable reduction is obtained in reflectory halation effects.

60. In Figure 5, I have illustrated a typical bi-pack material, according to the last-mentioned modification. All of the layers I<sub>c</sub>, II<sub>c</sub> and III<sub>c</sub> are supported between the front and back supports A and B. The layers I<sub>c</sub> and II<sub>c</sub> are poured one on the other and carried by support A, while the layer III<sub>c</sub> is carried by support B. The layer I<sub>c</sub> is a non-sensitized, i. e., merely blue-sensitive silver halide layer, preferably silver bromide gelatine. This layer may contain a dyestuff-forming substance as set forth in connection with the colorless layers illustrated in Figures 1, 2 and 3. The layer II<sub>c</sub> may also be a silver bromide layer containing a yellow dyestuff, for example, the potassium salt of chrysophenine G (Schultz

304). This yellow layer is sensitized for green with, for example thiopseudocyanin. The layer III<sub>c</sub> is a red-sensitive emulsion which contains a red or a purple-red dyestuff, such for example as Benzo Fast Scarlet 4 BS or Diamine Fast Pink G. 5

Figure 6 represents a relative arrangement of colors and sensitivities, the same as in Figure 5, the only difference being that in this case, layer I<sub>d</sub> which is the colorless blue-sensitive layer, is carried by the front support and layers II<sub>d</sub> and III<sub>d</sub> are carried by the back support B.

The relative order and arrangement of the colors and sensitivities in the layers as well as the position of the support with respect to the layers are merely set forth by way of example. One 15 may employ any suitable colors or dyestuff-forming substances resulting in colors, providing only that colors utilized are complementary to the sensitization of the corresponding layer in the copying material, and that they transmit light 20 for which the layer itself is sensitive as well as the layer situated thereunder.

It will be further understood that one might employ four part-images instead of three part-images, as set forth in the above examples. In this case the layers are sensitized in such a fashion that the part images may be obtained for four-color photography, the fourth part-image being employed either for the production of a black part-image or key-print, or of a fourth 25 colored part-image. For example, two colored part-images might be obtained in respect to the green spectral zone. In such a case, one layer would be sensitive, for example, to blue, one for blue-green, one for yellow-green and one for red. The use of dyestuffs in the predyed layers of the exposure material, which dyestuffs act both as filter dyestuffs and for the formation of the master image, depends likewise in this case on the sensitization of the copying material. In such 40 case, if a bi-pack material is used, such as that shown in Figure 5, two of the light-sensitive layers are carried on each support and it is possible to obtain sharp images even with this larger number of part-images. 45

I claim as my invention:

1. A material for color photography comprising at least three superposed silver halide emulsion layers, each of which is sensitive to one of three primary colors including a colorless silver 50 halide front layer predominantly sensitized to the blue spectral region and substantially insensitive to the other primary colors, a second silver halide layer predominantly sensitized for one of the other primary colors and colored yellow 55 by a dyestuff which is not removable by ordinary photographic treating baths but which is selectively removable under the influence of the photographic image and which transmits light for which the third layer is sensitive, and a third silver halide layer predominantly sensitized for the remaining primary color but effectively insensitive to light for which the second layer is predominantly sensitized and which is transmitted therethrough, the light transmission characteristic of said material being such that all of said layers can be exposed from the front of said material to light for which they are predominantly sensitive.

2. A material for color photography comprising at least three superposed silver halide emulsion layers, each of which is sensitive to one of three primary colors including a colorless silver halide front layer predominantly sensitized to the blue spectral region and substantially in- 70 75

- 5 sensitive to the other primary colors, a second silver halide layer predominantly sensitized for one of the other primary colors and colored yellow by a dyestuff which is not removable by ordinary photographic treating baths but which is selectively removable under the influence of the photographic image and which transmits light for which the third layer is sensitive, and a third silver halide layer predominantly sensitized for 10 the remaining primary color and colored by a dyestuff which is not removable by ordinary photographic treating baths but which is selectively removable under the influence of the photographic image and which absorbs light rays for 15 which the yellow layer is sensitized, the light transmission characteristic of said material being such that all of said layers can be exposed from the front of said material to light for which they are predominantly sensitive.
- 20 3. A material for color photography comprising at least three superposed silver halide emulsion layers each of which is sensitive to one of three primary colors including a colorless silver halide front layer containing a colorless dye- 25 stuff forming substance and being predominantly sensitized to the blue spectral region and substantially insensitive to the other primary colors, a second silver halide layer predominantly sensitized for one of the other primary colors 30 and colored yellow by dyestuff which is not removable by ordinary photographic treating baths but which is selectively removable under the influence of the photographic image and which transmits light for which the third layer is sensitive, and a third silver halide layer predominantly 35 sensitized for the remaining primary color but effectively insensitive to light for which the second layer is predominantly sensitized and which is transmitted therethrough, the light 40 transmission characteristic of said material being such that all of said layers can be exposed from the front of said material to light for which they are predominantly sensitive.
4. A multi-pack material for color photography 45 comprising two transparent supports and at least three silver halide emulsion layers, each of which is sensitive to one of three primary colors including a colorless layer predominantly sensitized for the blue spectral region coated on the front support and substantially insensitive to the other primary colors, a second layer predominantly sensitized for one of the other primary colors and colored yellow by a dyestuff which is not removable by ordinary photographic treating 50 baths but which is selectively removable under the influence of the photographic image and which transmits light for which the third layer is sensitive, said second layer being coated on one of the two supports and located between the colorless layer and the third layer which is predominantly sensitive to the remaining primary color but effectively insensitive to light for which the second layer is predominantly sensitized and which is transmitted therethrough, said third 55 layer being coated on the rear support, the light transmission characteristic of said material being such that all of said layers can be exposed from the front of said material to light for which they are predominantly sensitive.
- 60 5. A multi-pack material for color photography comprising two transparent supports and at least three silver halide emulsion layers, each of which is sensitive to one of three primary colors including a colorless layer predominantly sensitized for the blue spectral region coated on the front support, said layer being substantially 65 insensitive to the other primary colors, a predominantly green sensitive silver halide emulsion colored yellow by a dyestuff which is not removable by ordinary photographic treating baths but which is selectively removable under the influence of the photographic image and which transmits light for which the third layer is sensitive coated on the rear of the first support, and a predominantly red sensitive silver halide emulsion colored red by a dyestuff which is not removable by ordinary photographic treating 70
- 75

front support and substantially insensitive to the other primary colors, a second layer predominantly sensitized for one of the other primary colors and colored yellow by a dyestuff which is not removable by ordinary photographic treating baths but which is selectively removable under the influence of the photographic image and which transmits light for which the third layer is sensitive, said second layer being coated on one of the two supports and located between the colorless layer and the third layer which is predominantly sensitive to the remaining primary color, said third layer being colored by a dyestuff which is not removable by ordinary photographic treating baths but which is selectively removable under the influence of the photographic image and which absorbs light rays for which the yellow layer is sensitive, said third layer being coated on the rear support, the light transmission characteristic of said material being such that all of said layers can be exposed from the front of said material to light for which they are predominantly sensitive.

6. A material for color photography comprising at least three superposed silver halide emulsion layers including a colorless silver halide front layer predominantly sensitized for the blue spectral region and substantially insensitive to the other primary colors, a second silver halide layer predominantly sensitized for green and colored yellow by a dyestuff which is not removable by ordinary photographic treating baths but which is selectively removable under the influence of the photographic image and which transmits light for which the third layer is sensitive, and a third silver halide layer predominantly sensitized for red but effectively insensitive to light for which the second layer is predominantly sensitive and which is transmitted therethrough, the light transmission characteristic of said material being such that all of said layers can be exposed from the front of said material to light for which they are predominantly sensitive.

7. A material for color photography comprising at least three superposed silver halide emulsion layers including a colorless silver halide front layer predominantly sensitized for the blue spectral region and substantially insensitive to the other primary colors, a second silver halide layer predominantly sensitized for green and colored yellow by a dyestuff which is not removable by ordinary photographic treating baths but which is selectively removable under the influence of the photographic image and which transmits light for which the third layer is sensitive, and a third silver halide layer predominantly sensitized for red and colored red by a dyestuff which is not removable by ordinary photographic treating baths but which is selectively removable under the influence of the photographic image.

8. A multi-pack material for color photography comprising a colorless predominantly blue sensitive silver halide emulsion layer on the front of the first support, said layer being substantially insensitive to the other primary colors, a predominantly green sensitive silver halide emulsion colored yellow by a dyestuff which is not removable by ordinary photographic treating baths but which is selectively removable under the influence of the photographic image and which transmits light for which the third layer is sensitive coated on the rear of the first support, and a predominantly red sensitive silver halide emulsion colored red by a dyestuff which is not removable by ordinary photographic treating

baths but which is selectively removable under the influence of the photographic image coated on the front of the second support.

9. A multi-pack material for color photography comprising a colorless predominantly blue sensitive silver halide emulsion layer containing a colorless dye-forming material on the front of the first support said layer being substantially insensitive to the other primary colors, a predominantly green sensitive silver halide emulsion colored yellow by a dyestuff which is not removable by ordinary photographic treating baths but which is selectively removable under the influence of the photographic image and which transmits light for which the third layer is sensitive coated on the rear of the first support, and a predominantly red sensitive silver halide emulsion colored red by a dyestuff which is not removable by ordinary photographic treating baths but which is selectively removable under the influence of the photographic image coated on the front of the second support.

10. A material for color photography comprising at least three superposed silver halide emulsion layers including a colorless silver halide front layer predominantly sensitized for the blue spectral region and substantially insensitive to the other primary colors, a second silver halide layer predominantly sensitized for green and colored yellow by a dyestuff which is not removable by ordinary photographic treating baths but which is selectively removable under the influence of the photographic image and which transmits light for which the third layer is sensitive, and a third silver halide layer predominantly sensitized for red and colored yellow by a dyestuff which is not removable by ordinary photographic treating baths but which is selectively removable under the influence of the photographic image.

11. A multi-pack material for color photography comprising a plurality of differently sensitized silver halide emulsion layers supported face to face between a pair of supports, one of said layers being a colorless blue sensitive layer which is substantially insensitive to the other primary colors, said one layer being supported on the support through which exposure light initially passes, the second one of said layers being predominantly sensitized for one of the other primary colors and colored yellow by a dyestuff which is not removable by ordinary photographic treating baths but which is selectively removable under the influence of a silver image, the third one of said layers being predominantly sensitive to the remaining primary color but effectively insensitive to light for which the second layer is predominantly sensitized and which is transmitted therethrough, the light transmission characteristic of said material being such that all of said layers can be exposed from the front of said material to light for which they are predominantly sensitive.

12. A multi-pack material for color photography comprising a plurality of differently sensitized silver halide emulsion layers supported face to face between a pair of supports, one of said layers being a colorless blue sensitive layer having a dyestuff forming substance incorporated therein and being substantially insensitive to the other primary colors, said one layer being supported on the support through which exposure light initially passes, the second one of said layers

being predominantly sensitized for one of the other primary colors and colored yellow by a dyestuff which is not removable by ordinary photographic treating baths but which is selectively removable under the influence of a silver image, the third one of said layers being predominantly sensitive to the remaining primary color but effectively insensitive to light for which the second layer is predominantly sensitized and which is transmitted therethrough, the light transmission characteristic of said material being such that all of said layers can be exposed from the front of said material to light for which they are predominantly sensitive.

13. A multi-pack material for color photography comprising a colorless predominantly blue sensitive silver halide emulsion layer on the front of the first support, said layer being substantially insensitive to the other primary colors, a predominantly green sensitive silver halide emulsion colored yellow by a dyestuff which is not removable by ordinary photographic treating baths but which is selectively removable under the influence of the photographic image and which transmits light for which the third layer is sensitive coated on the rear of the first support, and a predominantly red sensitive silver halide emulsion coated on the front of the second support, the light transmission characteristic of said material being such that all of said layers can be exposed from the front of said material to light for which they are predominantly sensitive.

14. A material for color photography comprising at least three superposed silver halide emulsion layers, including a light sensitive silver halide front layer which transmits blue, green, and red light and is predominantly sensitive to one of these primary colors, a second silver halide layer which is colored by a dyestuff which is not removable by ordinary photographic treating solutions but which is selectively removable under the influence of the photographic image, the dyestuff absorbing the light of the primary color for which the front layer is predominantly sensitive but transmitting the light of the two other primary colors, the layer being predominantly sensitized to one of these two colors and a third silver halide layer which is transmittant for and predominantly sensitized to the remaining primary color but effectively insensitive to light for which the second layer is sensitized, the light transmission characteristic of said material being such that all of said layers can be exposed from the front of said material to light for which they are predominantly sensitive.

15. The method of producing a subtractive multi-color picture from a multi-layer light sensitive silver halide material, having on a common support a colorless surface layer of silver halide emulsion and a differently sensitized silver halide layer which is uniformly pre-dyed by a reducible dyestuff resistant to the ordinary photographic treating solutions but capable of being locally destroyed under the control of a metallic silver image, which comprises exposing each of said layers to light to form latent images in the silver halide layers, developing the latent images to form silver images, coloring the colorless surface layer uniformly with a reducible dyestuff which transmits blue light and thereafter destroying the dyestuff in the surface layer and the pre-dyed layer at the points of metallic silver.

BÉLA GASPAR.